

# UNITED STATES PATENT OFFICE.

SAMUEL M. COOPER, OF MCKEESPORT, PENNSYLVANIA, ASSIGNOR TO AMERICAN SHEET & TIN PLATE COMPANY, OF PITTSBURG, PENNSYLVANIA, A CORPORATION OF NEW JERSEY.

## METHOD OF MAKING PLANISHED SHEET-IRON.

No. 918,971.

Specification of Letters Patent. Patented April 20, 1909.

Application filed November 21, 1908. Serial No. 463,798.

To all whom it may concern:

Be it known that I, SAMUEL M. COOPER, of McKeesport, Allegheny county, Pennsylvania, have invented a new and useful Method 5 of Making Planished Sheet-Iron, of which the following is a full, clear, and exact description.

My invention relates to the manufacture of planished sheet iron, which presents a mottled polished appearance in the finished sheets. Heretofore the common practice in producing this material has been to finish the 10 packs of sheets in the ordinary manner and then produce indentations in the sheets 15 by hammering them in sets of about a half a dozen sheets between dies which have a mottled surface. This hammering action not only mottles the sheets, but also polishes them. It has also been proposed to mottle 20 the sheets by rolling after the sheets have been brought to substantially their finished gage and before they are hammered in plain dies.

I have discovered that by machining the 25 mottled surface on iron rolls made of a dense mixture of iron, I can reduce the sheets in packs immediately after matching and at the same time mottle the sheets; so that they may be hammered and polished between 30 plain dies and an improved product obtained. I have also found that by this improved method I can hammer and polish a very much larger number of sheets than was heretofore possible; using about 60 to 75 35 sheets to the pack.

In carrying out my invention, I first roll the sheets singly and successively from the sheet bars in the ordinary manner, and I then form a pack of these sheets of usually from 40 three to five in number, the sheets of the pack being reheated to the proper temperature. Previous to piling the broken-down pairs of sheet bars are preferably dipped in a solution of charcoal dust and water in order 45 to prevent the sheets from sticking in the packs. When the packs of reheated sheets are prepared, they are reduced to the desired gage by successive passes through a single pair of mottle rolls. These mottle rolls are 50 preferably prepared in accordance with the

process described in my co-pending application Serial No. 463797 filed November 21st, 1908—that is, the surface of these rolls is pock-marked by means of a steel-forming roller having raised projections upon it which is forced against the surface of the iron roll. The pack of three to five sheets when thus reduced in the mottle rolls will present a mottled appearance, the sheets of the pack are then taken apart, and the ends are 55 sheared. The sheets are then pickled, and the partially reduced sheets are also preferably pickled prior to reheating and mottling. After pickling the mottled sheets, the dried sheets are then piled into packs of 60 to 75 in 60 number. In this act of piling charcoal dust is also preferably supplied between the sheets. The pile is then preferably inclosed in loose 65 sheets which are wired about the back as an envelop, extra cover sheets being supplied at 70 the top and bottom of the pack. The package is then put in a baking furnace and heated to the proper temperature and is then taken to the brooms. Each sheet is then broomed 75 on both sides, and the pack is repiled and taken to the hammer dies for leveling. These dies act to flatten and level the sheets. The top and bottom cover sheets are retained on the pile and the pile is then reheated and taken to the hammers. These hammer dies 80 have plain surfaces, and the pile is then hammered in the usual manner between these dies to polish the sheets.

The advantages of my invention result 85 from the use of the pock-marked rolls for rolling the matched packs to their final gage; in connection with the polishing by smooth-faced hammers, I thereby secure economy in the process owing to the large number of sheets in the pile which may be hammered 90 at the same time, and I also produce an improved product.

Variations may be made in the form and arrangement of the apparatus without departing from my invention.

I claim:

1. The method of making planished sheet iron, consisting in rolling singles on plain rolls, piling the sheets into packs, and rolling the packs down to the desired gage on mot- 100

tled rolls while in a heated condition, and then hammering a plurality of the sheets between plain dies; substantially as described.

2. The method of making planished sheet iron, consisting in rolling singles on plain rolls, piling the sheets into packs and rolling the packs down to the desired gage on mottled rolls while in a heated condition, and then repiling the sheets into piles of a larger

number and hammering the said piles of 10 sheets between plain dies; substantially as described.

In testimony whereof, I have hereunto set my hand.

SAMUEL M. COOPER.

Witnesses:

J. H. RUILOBA,  
G. C. KIMBALL.